

## UNITED STATES PATENT OFFICE

2,002,106

## PROCESS FOR TREATING VEGETABLE FIBERS

Albert Bodmer and Ernst Weiss, Wattwil, Switzerland, assignors to Heberlein Patent Corporation, New York, N. Y., a corporation of New York

No Drawing. Application August 10, 1932, Serial No. 628,184. In Germany March 17, 1932

8 Claims. (Cl. 8—20)

This invention relates to a method of treating vegetable fibrous material and to the resulting product.

The principal object of the invention is to produce an improved permanent finish of such material in a simple efficient manner. Further objects and advantages of the invention will more fully appear from the following description wherein certain preferred ways of carrying out the invention are set forth. The invention will be more particularly pointed out in the appended claims.

Valuable effects can be produced on vegetable fibers by the action of cuprammonium solution and caustic alkali solution in accordance with the procedure of applicant's copending application which has now matured into Patent #1,896,620 dated February 7, 1933. That process rests upon the production of a swelling effect initially produced in a certain manner upon the fibers with a following treatment thereof whereby alteration of the properties of the fibrous structure is produced. It has now been discovered in accordance with this invention that a very small addition of free alkali sharply increases the swelling of the material and cessation of swelling (Entquellung) may be arranged so that the ennobling effect on the fiber is considerably improved. I have found also in accordance with this invention that the addition and incorporation of the alkali furthermore permits a very considerable decrease, to about one-half, of the amount of ammonia required in the cuprammonium solution. The addition of alkali must be small so that the amount of free alkali contained in the solution will not exceed 1.5%. In actual practice it is preferable to work with an amount of free alkali hydroxide of 0.5-1%. For this purpose caustic soda is employed as alkali although caustic potash and the hydroxides of the rare earth metals are also useful.

The cuprammonium solution thus made is capable by itself of ennobling vegetable fibers and to produce effects of the kind described in the copending application Ser. No. 321,505, now Patent No. 1,896,620 above referred to, whereby as a rule somewhat less stiffening is caused but greater elasticity than obtainable by the procedure of the copending application mentioned, is secured. The discontinuance of swelling of the fiber according to the kind of effect desired can be obtained with water, dilute acid or dilute alkali lye, whereby generally the effect produced by the dilute alkali is stiffer, that with dilute acid

is softer; whereas the effect produced by water lies intermediate these two effects.

If one employs activated cuprammonium solution (containing a small quantity of free caustic alkali) followed by treatment with alkali, one obtains half stiff or stiff, as well as linen-like effects, which are intensified as compared with the effects secured by the process of the copending application mentioned. These effects according to the present process are secured with decreased ammonia consumption, the copper content remaining unchanged, with the consequence that the process is greatly improved from the viewpoint of economy and profit.

The novel method of the present invention is useful for all kinds of vegetable fibrous structures as well as loose fibers. Vegetable fibrous material may be submitted to treatment in the bleached state or in any other pre-treated condition as well as mercerized. Fibrous structures consisting of vegetable fibers of various origins or mixed with other natural or artificial fibers, can be ennobled in this manner. By the aid of suitable apparatus the same process can be carried out so that by the action of the swelling material the fibrous structure is not altered throughout, but the swelling occurs only on one side and superficially. The action not only of the cuprammonium but also of the alkali lye may be carried on while the fibers are in either loose or tensioned condition. The ennobled fibrous structures, owing to their plastic properties, are very adaptable to subsequent mechanical treatment; for instance, by calendering and the like, extraordinarily supple (geschmeidige) effects are produced.

By the novel method here disclosed, it is also possible to obtain patterning by local action of the swelling agents. For this purpose it is possible to employ direct application by printing, spraying or splattering with or without the use of thickeners as well as to use resist printing accompanied by subsequent dipping in to the swelling agent. In addition, durable patterns can be produced by subjecting a previously mercerized fabric to local hot pressing and then subjecting it to the action of swelling agents in accordance with the present procedure.

It has been previously suggested to obtain ennoblement by the action of cuprammonium solution containing a substantial amount of free alkali, always more than 1.5-2% free alkali. However, solutions of this kind are not capable of producing the ennobling effects above referred to because they cause a noticeable solvent action on the cellulose subjected to swelling so that the

precipitation phenomenon herein described and occurring in the course of the process for eliminating the swelling does not appear. Further the stability of cuprammonium solutions having high alkali content, is limited.

The following are examples of the process employed, these examples being given simply as illustrations. It is to be understood that the invention is not restricted thereto.

10

*Examples*

1. Bleached cretonne fabric of cotton is impregnated with a cuprammonium solution containing 15 grams of copper and 5 grams of sodium hydroxide per liter and after a short action time of 15 seconds is precipitated by sulfuric acid of 2° Bé. at 15° C. Coincidentally with the acid precipitation the elimination from the fiber of the copper is assured. After calendering the finished fabric exhibits a supple elastic feel resembling linen.

2. Mercerized cotton yarn is briefly treated during 15 seconds with a solution of cuprammonium containing 12 grams of copper and 8 grams of potassium hydroxide per liter and immediately thereafter washed with water at 18° C. Elimination of copper is accomplished in the usual way with dilute acid. The finished yarn resembles linen yarn.

3. Pre-treated calico fabric is passed for a short time through a cuprammonium solution containing 10 grams of copper and 3 grams of sodium hydroxide per liter, after an air passage of 40 seconds, followed by precipitation by the aid of dilute caustic soda at 4° Bé. at 20° C. Elimination of copper after the latter treatment is effected in the usual manner. The result of the ennobling effect is similar to that in Example 1 except that an increased stiffness is noted.

4. Cuprammonium solution comprising 13 grams of copper and 10 grams of sodium hydroxide per liter is caused to act upon a heavy cotton fabric for 20 seconds at 10° C. Immediately thereafter the swollen unwashed fabric is mercerized in the mercerizing machine with the use of concentrated soda lye, followed by elimination of copper by acidulation and washing. For finishing intense calendering and mangling are applied with the result that the fabric assumes the characteristics of heavy linen.

5. A resist-printed fabric is treated according to the procedure in Example 4. The fabric exhibits patterning of damask-like nature; the reserve portions of the fabric show unaltered properties, and thus contrast with the other parts that have been subjected to the action of cuprammonium solution.

6. Card sliver made of ramie fibers is impregnated with a solution of cuprammonium containing 14 grams of copper and 4 grams of sodium hydroxide per liter and after a reaction

time of 30 seconds then subjected to mercerizing with soda lye and is de-coppered in the usual manner. After drying there results a lustrous stiff fiber of agglutinated ramie fibers or filaments.

Thus while we have described our improvements in detail and with respect to certain preferred forms, we do not desire to be limited to such details or forms since, as will be understood by those skilled in the art after understanding our invention, many changes and modifications may be made and the invention embodied in widely different forms without departing from the spirit and scope thereof in its broader aspects, and we desire to cover all modifications, forms and embodiments coming within the scope of any one or more of the appended claims.

Having thus described our invention, what we claim as new and desire to secure by Letters Patent, is:—

1. A method of producing permanent finish effects on vegetable cellulose material which comprises preparing a bath containing cuprammonium and a free alkali metal hydroxide in which the percentage of free alkali does not exceed 1.5% of the weight of the solution, swelling the vegetable cellulose material by subjecting it to the bath and subjecting the so-treated material to an agent for interrupting the swelling action of said solution.

2. The method according to claim 1 in which the amount of free alkali is from 0.5 to 1%.

3. The method according to claim 1 in which the interruption of the swelling is effected by dilute acid.

4. The method according to claim 1 in which the swelling is interrupted by treatment with water.

5. The method according to claim 1 in which the swelling is interrupted by treatment with dilute alkali lye.

6. The method according to claim 1 in which the interruption of swelling is effected by treating the fibrous materials after treatment with the alkaline cuprammonium solution with concentrated alkali lye of a strength to cause mercerization thereof.

7. The method according to claim 1 in which the alkaline cuprammonium solution acts on the material to form a pattern.

8. Steps in the method of producing permanent finish effects on vegetable cellulose material which consist in preparing a cuprammonium solution containing a free alkali metal hydroxide in which the percentage of free alkali does not exceed 1.5% of the weight of the solution, and subjecting the vegetable cellulose material to said solution.

ALBERT BODMER.  
ERNST WEISS.